

[54] A PHOTOGRAPHIC COMPOSITION OF  
1,1-BIS-SULFONYL ALKANE AND  
HYDROXYLAMINE

[75] Inventors: Donald G. Yungkurth; Gary J.  
McSweeney, both of Rochester, N.Y.

[73] Assignee: Eastman Kodak Company,  
Rochester, N.Y.

[22] Filed: Oct. 1, 1971

[21] Appl. No.: 185,830

[52] U.S. Cl..... 96/29 R, 96/94, 96/109

[51] Int. Cl..... G03c 5/54

[58] Field of Search..... 95/109, 29

[56] References Cited

UNITED STATES PATENTS

3,647,453 3/1972 Haist et al..... 96/109

3,293,034 12/1916 Green et al..... 96/61 X

Primary Examiner—Norman G. Torchin

Assistant Examiner—John L. Goodrow

Attorney—Robert W. Hampton et al.

[57]

ABSTRACT

A combination of 1,1-bis-sulfonyl alkane silver halide solubilizing agent with a hydroxylamine silver halide developing agent in a photographic chemical transfer process, element, composition and/or product provides a developed image having increased stability, with low minimum density, increased maximum density and desired sensitometric properties. This combination can include addenda commonly employed in photographic processing compositions and elements.

13 Claims, No Drawings

**A PHOTOGRAPHIC COMPOSITION OF  
1,1-BIS-SULFONYL ALKANE AND  
HYDROXYLAMINE**

**BACKGROUND OF THE INVENTION**

**1. Field of the Invention**

This invention relates to photographic processing compositions, elements and processes. In one of its aspects it relates to photographic processing compositions containing a combination of a 1,1-bis-sulfonyl alkane silver halide solubilizing agent with a hydroxylamine silver halide developing agent to provide improved developed images. In another of its aspects it relates to photographic elements and processes employing the described combination in a silver salt diffusion transfer system.

**2. Description of the State of the Art**

In recent years photographic chemical transfer processes, elements and compositions have become well known. Briefly, the commonly employed chemical transfer process is characterized by the use of a photographic emulsion layer and an image receiver or silver precipitating layer contiguous to the photographic emulsion layer. After exposure of the photographic layer, a processing composition is applied between the exposed photographic layer and the silver precipitating layer. The processing composition usually contains a silver halide solvent which causes the unexposed silver salts, usually silver halides, to form a silver complex which diffuses to the image receiver or silver precipitating layer where development nuclei or precipitating agent within that layer causes the silver to be precipitated from the silver complex. Development nuclei can be present in the image receiving layer before contact with the complex or the nuclei can be formed in situ. Diffusion transfer photographic systems are described, for example, in U.S. Pat. No. 2,698,237 of Land issued Dec. 28, 1954; U.S. Pat. No. 2,647,056 of Land issued July 28, 1953; U.S. Pat. No. 3,108,001 of Green issued Oct. 22, 1963; and U.S. Pat. No. 3,345,166 of Land issued Oct. 3, 1967. The processing composition employed in a chemical transfer system normally contains a silver halide solubilizing agent and a silver halide developing agent and is usually applied as a viscous fluid layer spread between the photosensitive layer and the image receiving layer.

Likewise, silver halide complexing agents have been employed in monobaths wherein a single processing composition can be utilized to both develop and fix or stabilize a photographic silver halide emulsion layer. Such compositions contain a silver halide developing agent in addition to the silver halide solubilizing agent.

Many compounds have been tried as silver halide solubilizing or complexing agent in the described systems. One commonly employed silver halide solubilizing or complexing agent employed is sodium-thiosulfate pentahydrate. Other silver halide solubilizing or complexing agents which have been employed include potassium thiocyanate and certain mercaptans such as mercapto acetic acid. These and other silver halide solubilizing or fixing agents have not been found satisfactory when employed with hydroxylamine silver halide developing agents due to the production of undesired maximum and minimum density in the developed image. This is illustrated in the following comparative examples, 2, 3, 4, 5 and 6.

The requirements for developing agents to be employed with the described silver halide complexing agents in a chemical transfer system to provide the desired stable image are very stringent and relatively few of the developing agents which are satisfactory for general silver halide developing systems will be satisfactory or sufficiently active for chemical transfer systems. Commonly employed developing agents include hydroquinone, pyrocatechol, araboascorbic acid, or a reductone developing agent such as dihydro anhydro piperidino hexose reductone. Although such developing agents will produce a positive image in a chemical transfer system when employed with certain silver halide complexing agents, they provide less than desired maximum and minimum densities. This is illustrated in the following comparative Examples 7 and 8.

Thus, there has been a continuing need for a combination of a silver halide complexing agent with a silver halide developing agent which provides improved maximum and minimum densities and developing action with improved developed image stability and without objectionable stain on a processed print.

**SUMMARY OF THE INVENTION**

According to the invention it has been found that desired increased maximum and minimum density without undesired oxidation stain, and with improved developed image stability can be provided in a chemical transfer system employing a combination of a 1,1-bis-sulfonyl alkane silver halide solubilizing agent with a hydroxylamine silver halide developing agent.

This combination of silver halide complexing agent with a hydroxylamine silver halide developing agent provides excellent silver halide solubilizing or fixing properties and developing properties in a range of photographic processes and products wherein silver halide solvents and developing agents are ordinarily employed in combination. This combination can be employed with an auxiliary silver halide developing agent.

**DETAILED DESCRIPTION OF THE INVENTION**

A range of the described 1,1-bis-sulfonyl alkanes, also known as beta-disulfones, can be employed in combination with a hydroxylamine silver halide developing agent according to the invention. The beta-disulfones and their chemical reactions have been described in the literature. For example, the preparation of these compounds and reactions in which they are involved are described in Suter, *ORGANIC CHEMISTRY OF SULFUR*, pages 735 and 739. Of the class of beta-disulfone compounds, however, it has been found that particular beta-disulfones, such as 1,1-bis-sulfonyl alkanes are excellent silver halide solvents with hydroxylamine silver halide developing agents. Suitable 1,1-bis-sulfonyl alkanes employed according to the invention can be represented by the formula



wherein  $R_1$  and  $R_2$  each represent an alkyl group containing one to four carbon atoms and  $R_3$  represents hydrogen or an alkyl group containing one to four carbon atoms. The term alkyl as employed herein also includes substituted alkyl groups and preferably substituted lower alkyl group containing from one to four carbon atoms. Substituted alkyl groups include hydroxyalkyl

groups, e.g., hydroxyethyl or hydroxybutyl; alkoxyalkyl group such as methoxyethyl or butoxybutyl; carboxyalkyl such as a carboxyethyl or carboxybutyl; sulfoalkyl such as a sulfoethyl or sulfobutyl; sulfatoalkyl such as a sulfatoethyl or sulfatobutyl; an acyloxyalkyl such as beta-acetoxyethyl or butyloxybutyl; or alkoxy carbonylalkyl such as a beta-methoxycarbonylethyl or ethoxy carbonylbutyl.

1,1-Bis-sulfonyl alkanes within the described formula include, for example, 1,1-bis-(methylsulfonyl)ethane; 1,1-bis-(ethylsulfonyl)-ethane; 1,1-bis-(methylsulfonyl)-propane; 1-ethylsulfonyl-1-methylsulfonylmethane; 1-ethylsulfonyl-1-methylsulfonyl ethane and the like. Especially useful 1,1-bis-sulfonyl alkanes are bis(methylsulfonyl)methane, bis(ethylsulfonyl)methane, bis(beta-hydroxyethylsulfonyl)methane, bis(carboxymethylsulfonyl)methane, and bis(beta-carboxyethyl-sulfonyl)-methane.

A range of hydroxylamine silver halide developing agents can be employed in the described combination also. Useful hydroxylamine silver halide developing agents include, for example, compounds of the formula:



wherein  $R_4$  and  $R_5$  are each, individually, hydrogen, alkyl containing one to four carbon atoms, alkoxyalkyl containing three to six carbon atoms, or alkoxyalkoxyalkyl containing five to 10 carbon atoms. Typical hydroxylamine silver halide developing agents within this formula include hydroxylamine, N-methylhydroxylamine, N-ethylhydroxylamine, N-propylhydroxylamine, N-isopropylhydroxylamine, N,N-diethylhydroxylamine, N,N-dimethylhydroxylamine, N-methyl-N-propylhydroxylamine, N-methyl-N-isopropylhydroxylamine, N-ethyl-N-n-propylhydroxylamine, N,N-diisopropylhydroxylamine, N,N-di-n-propylhydroxylamine, N-ethyl-N-methylbutylhydroxylamine, N-methyl-N-isobutylhydroxylamine, N-ethyl-N-hydroxyethylhydroxylamine, N-hydroxyethyl-N-carboxyethylhydroxylamine, N,N-di-(methoxyethyl)-hydroxylamine, N,N-di-(2-ethoxyethyl)hydroxylamine, N,N-di-(2-methoxyethoxyethyl)hydroxylamine, and the like. Hydroxylamine silver halide developing agents are set out, for example, in U.S. Pat. No. 2,857,276 of Land et al., issued Oct. 21, 1958; U.S. Pat. No. 2,857,275 of Land et al., issued Oct. 21, 1958 and U.S. Pat. No. 2,857,274 of Land et al., issued Oct. 21, 1958, as well as a Netherlands Pat. No. 7015734 of Gevaert-Agfa; U.S. Pat. No. 3,343,958 of Morse, issued Sept. 26, 1967; British Pat. No. 902,314 of Polaroid, published Aug. 1, 1962; U.S. Pat. No. 3,287,124 of Green et al., issued Nov. 22, 1966; U.S. Pat. No. 3,287,125 of Green et al., issued Nov. 22, 1966; U.S. Pat. No. 3,293,034 of Green et al., issued Dec. 20, 1966; U.S. Pat. No. 3,362,961 of Green et al., issued Jan. 9, 1968; British Pat. No. 1,142,134 of Polaroid, published Feb. 5, 1969; U.S. Pat. No. 3,455,916 of Green et al., issued July 15, 1969; U.S. Pat. No. 3,467,711 of Bader et al., issued Sept. 16, 1969 and the like.

One embodiment of the invention is accordingly a photographic processing composition comprising a 1,1-bis-sulfonyl alkane silver halide solubilizing agent with a hydroxylamine silver halide developing agent, as de-

scribed. Such a processing composition is typically an aqueous alkaline processing composition.

Various development activators can be employed in combination with the described beta-disulfone silver halide solubilizing agent and hydroxylamine silver halide developing agent. These include any of those which provide the desired activation of the described developing agents and desired silver halide solvent activity. These include, for example, alkaline development activators, such as inorganic alkalies including,

10 for example, sodium hydroxide, potassium hydroxide, cesium hydroxide and/or lithium hydroxide; alkali metal carbonates, such as sodium carbonate, and potassium carbonate; alkali metal phosphates, such as tri-

15 sodium phosphate and/or organic alkaline development activators, such as quaternary ammonium bases and salt, such as amino alkanols and similar alkaline materials and/or alkali releasing materials. In some instances the described hydroxylamine silver halide de-

20 veloping agent is alkaline and contributes to the alkalinity of the processing composition.

The described silver halide solubilizing agents can be utilized in a photographic processing composition in a concentration of at least about 1 gram of disulfone per

25 liter of processing composition. The concentration of such silver halide solubilizing agents can vary over a wide range depending on the particular components of the processing composition, the desired image, the particular photographic silver halide emulsion employed,

30 processing conditions and the like. Generally, however, the concentration of described disulfone utilized will vary between about 0.1 and about 1.0 moles of the described 1,1-bis-sulfonyl alkane silver halide solubilizing agent per liter of processing composition.

35 When the described disulfones are employed in processing compositions for clearing or fixing silver halide in developed photographic elements, usually at least about 5 to 200 grams of the beta-disulfone is employed per liter of processing composition to obtain the fixing 40 within a practical time. Lower concentrations can be employed when the described disulfone is employed as a silver halide solubilizing agent in a silver salt chemical transfer system.

45 The described disulfone silver halide complexing agents provide fixing or clearing action in alkaline or basic compositions. Generally alkaline compositions have a pH of at least 8 or 9, and preferably at least about 11, are employed. However, the alkalinity of the processing compositions can vary over a wide range depending upon the particular photographic element processed, particular processing condition, the hydroxylamine silver halide developing agent employed, processing time and the like.

50 A range of concentration of the described hydroxylamine silver halide developing agent can be employed in the combination according to the invention. A suitable concentration is typically about 0.10 mole to about 1.50 mole of hydroxylamine silver halide developing agent per liter of processing composition.

55 An especially useful processing composition is an aqueous alkaline photographic processing solution containing bis(methylsulfonyl)methane with N,N-diethylhydroxylamine.

60 While it is especially useful in a chemical transfer system to employ the described combination of disulfone silver halide solubilizing agent and hydroxylamine silver halide developing agent in a processing composi-

tion, such as an aqueous alkaline processing solution, the described combination can be employed in the practice of the invention in a range of physical locations in a photographic chemical transfer system. For instance, the disulfone silver halide solubilizing agent can be employed in one or more layers of a photographic element and/or in a processing composition, if desired. The optimum location will depend upon the desired image, processing conditions, particular photographic system and the like. An especially useful location for the hydroxylamine silver halide developing agent is also in an aqueous alkaline processing solution employed in a silver salt chemical transfer system as described.

When the described disulfones are present in a photographic element, such as in the silver halide emulsion layer and/or in a lay separate from the silver halide emulsion, the concentration suitable can be varied over a wide range depending, primarily, upon the concentration of silver halide present initially in the photosensitive element and the degree it is desired to dissolve or solubilize the silver halide. The fact that the described disulfones can be incorporated in a photosensitive element is an important characteristic of these compounds. Silver halide solubilizing agent commonly employed, such as sodium thiosulfate pentahydrate, cannot be successfully incorporated in a photographic element, especially in a photographic silver halide emulsion layer since it provides undesired silver halide solvent action upon contact with the silver halide. The described disulfones, on the other hand, are relatively inert at a pH range below about 8 or 9 and, therefore, can be coated as a component of a photographic element at the pH or below. The disulfones become active silver halide solvents above this pH range. Alkaline activation of the described disulfone silver halide solubilizing agents with the hydroxylamine silver halide developing agents thus can provide both silver halide developing activity and silver halide solvent activity.

Another embodiment of the invention accordingly is a photographic element comprising a support, photographic silver halide, a 1,1-bis-sulfonyl alkane silver halide solubilizing agent with a hydroxylamine silver halide developing agent. A typical photographic element comprises a support, photographic silver halide, bis(methylsulfonyl)methane with N,N-diethylhydroxylamine.

When employed in a photographic element, a concentration of the described disulfone can vary depending upon the components of the photographic element, processing condition and the like but is typically about 0.24 mole to about 4 moles of the described disulfone per mole of silver halide present in the photographic element. A suitable range of hydroxylamine silver halide developing agent in a photographic element with the disulfone can also vary depending upon the described factors but is typically about 0.24 moles to about 4 moles of hydroxylamine silver halide developing agent per mole of silver halide in the photographic element. The concentration of the disulfone and hydroxylamine silver halide developing agent which is most suitable will depend on the location in the photographic element, the concentration of silver halide to be dissolved and the like.

Accordingly, another embodiment of the invention is in a process for developing and stabilizing an image in a photographic element comprising a support and ex-

posed photographic silver halide by contacting the element with an alkaline photographic processing composition containing a silver halide solubilizing agent with a silver halide developing agent, the improvement which comprises employing a 1,1-bis-sulfonyl alkane as the silver halide solubilizing agent with a hydroxylamine developing agent as the silver halide developing agent. This photographic element can provide a means for rapid access processing.

If desired, an alkaline solution containing conventional silver halide developing agents can be employed for activating the described hydroxylamine silver halide developing agent when employed in a photographic element. So-called web processing can be employed, as described, for example, in U.S. Pat. No. 3,179,517 of Tregillus et al issued Apr. 20, 1965 or so-called stabilization processing as described in Russell et al., PSA Journal, Volume 16B, Aug., 1950.

The time for processing a photographic element in the practice of the invention which includes developing a desired latent image can vary over a wide range typically between about 1 second to several minutes depending on the processing conditions, particular developing agents, particular silver halide solubilizing agent, desired image and the like.

The conditions for processing can also vary, but usually ambient pressures and temperatures of about 10°C. to about 40°C. are employed.

The described combination of disulfones with hydroxylamine silver halide developing agents are desirably employed in photographic chemical transfer systems, especially photographic silver salt chemical transfer systems. The described combination can be employed individually or in combination in one or more layers of photographic element and/or in a processing composition in such a system if desired. Suitable chemical transfer systems, processes, processing compositions and elements therefor are described, for example, in U.S. Pat. No. 2,452,181 of Land issued Feb. 27, 1951; U.S. Pat. No. 3,337,342 of Green issued Aug. 27, 1967, the disclosures of which are incorporated herein by reference. They can be used in so-called high speed diffusion transfer systems, processes and compositions therefor as described, for example, in U.S. Pat. No. 3,326,683 of Land et al. issued June 20, 1967; or in other types of chemical transfer systems such as described in U.S. Pat. No. 3,020,155 of Yackel issued Feb. 6, 1962; U.S. Pat. No. 2,584,030 of Land issued Jan. 29, 1952 and Belgian Pat. Nos. 749,931; 749,932; 749,933; 749,934; 749,935; and 749,930 published Oct. 16, 1970. These references are incorporated herein by reference and describe typical photographic products suitable for diffusion transfer systems comprising in combination (a) a photographic element comprising photographic silver halide, (b) a processing composition containing a silver halide solvent, typically in a rupturable container, and (c) an image receiving layer. Accordingly another embodiment of the invention is: in a photographic diffusion transfer product comprising in combination (a) a photographic element comprising photographic silver halide, (b) a processing composition comprising a silver halide solubilizing agent and (c) an image receiving layer, the product containing a silver halide developing agent, the improvement comprising a combination of 1,1-bis-sulfonyl alkane as the silver halide solubilizing agent and a hydroxylamine silver halide developing agent as the de-

scribed developing agent. The described combination of silver halide solubilizing agent and silver halide developing agent is preferably present in the processing composition.

The described combination of disulfone with hydroxylamine silver halide developing agent can be employed in a photographic silver salt diffusion transfer process comprising developing a latent image in a photographic diffusion transfer product comprising (a) a photographic element comprising photographic silver halide, (b) a processing composition comprising a silver halide solvent, and (c) an image receiving layer wherein the 1,1-bis sulfonyl alkane as described is employed as the silver halide solubilizing agent and a hydroxylamine is employed as the silver halide developing agent. More particularly this process can, for example, comprise the steps of exposing a photographic silver halide layer to form a latent image therein; developing the latent image with a processing composition, such as at a pH of about 12 to about 14, comprising the described hydroxylamine silver halide developing agent; contacting undeveloped silver halide in the photographic silver halide layer with a 1,1-bis sulfonyl alkane silver halide solvent to form an imagewise distribution of a silver complex in the unexposed areas of the photographic silver halide layer; transferring at least part of the silver complex to an image receiver layer contiguous to the photographic silver halide layer; reducing the silver complex in the presence of development nuclei to form a visible image in the receiver layer; and then, typically, lowering the pH of the processing composition to about 8 or below to form a stable developed image on the image receiver.

A wide variety of development nuclei or silver precipitating agents can be employed in diffusion transfer systems as described. These can be physical development nuclei or chemical precipitants including, for example, heavy metal in colloidal form and salts of these metals, salts of amines which form silver salts and/or non-diffusing polymeric materials with functional groups capable of combining with silver amines.

Suitable development nuclei and/or silver image precipitating agents within the described classes include metal sulfides, sulfonides, polysulfides, polyselenides, thiourea and its derivatives, stannous halides, sulfur, gold, platinum, palladium and mercury, colloidal silver sulfur, aminoguanidine sulfate, aminoguanidine carbonate, arsenous oxide, sodium stannate, hydrazines, xanthates and similar agents disclosed, for example, in U.S. Pat. No. 3,020,155 of Yackel et al. issued Feb. 6, 1962. A typical non-diffusing polymeric silver precipitant is poly (vinylmercaptoacetate). A range of concentration of development nuclei or silver precipitating agent can be employed. A concentration of the development nuclei or silver precipitant in the image receiving layer must be at least sufficient to insure the development of a positive image and sufficient removal of undeveloped silver salt from the light sensitive layer to be processed.

The described silver precipitating agents or development nuclei can be utilized in image reception layers that are separate elements from the light sensitive silver halide element processed or they can be utilized as reception layers integral with the light sensitive element. When the reception layer is integral with the light sensitive element, the reception layer is generally a sublayer over which is coated the silver halide in a vehicle that

is readily removable during processing, such as a hydrophilic colloid soluble in aqueous alkali such as cellulose ether phthalate.

Due to the inertness of the described disulfones, they can be incorporated in a receiving layer for chemical transfer systems. Again, the concentration of the disulfone can vary over a wide range depending on the concentration of the silver halide present in the system to be dissolved. The concentration can be about 0.25 to about 4 moles of described disulfone per mole of silver halide in the light sensitive element.

The described photographic element, receiving layers and/or processing compositions can also contain toning agents. Typical toning agents which can be employed include, for example, polyvalent inorganic salts as described in U.S. Pat. No. 2,698,236 of Land issued Dec. 28, 1954; silica as described in U.S. Pat. No. 2,698,237 of Land issued Dec. 28, 1954 and heterocyclic mercaptans such as mercaptoazoles, such as mercaptodiazoles, mercaptotriazoles, mercaptotetrazoles and corresponding selenazoles.

A processing composition employed in a diffusion transfer system as described is typically a viscous processing composition. A wide range of viscosity can be employed. The viscosity can be about 20 to about 100,000 centipoise typically about 100 to about 10,000 centipoise. Various thickening agents are suitable in the described processing compositions and processes of the invention. Any of those commonly employed in diffusion transfer photographic systems can be employed as well as those employed in viscous monobaths. These include those described, for example, in U.S. Pat. No. 3,120,795 of Land issued Feb. 11, 1964 such as hydroxyethylcellulose and carboxymethylcellulose.

The described combination of a 1,1-bis-sulfonyl alkane silver halide solubilizing agent with a hydroxylamine silver halide developing agent can be employed in combination with silver halide developing agents which are not hydroxylamines. The developing agents can be employed in such combinations as auxiliary developing agents or as the main component of a developing combination. Suitable silver halide developing agents which can be employed include, for example, polyhydroxybenzenes, such as hydroquinone silver halide developing agents, e.g., hydroquinone, alkyl-substituted hydroquinones as exemplified by tertiary butyl hydroquinone, methyl hydroquinone, 2,5-dimethyl hydroquinone and 2,6-dimethyl hydroquinone; catechols and pyrogallols; chloro-substituted hydroquinones, such as chlorohydroquinone or dichlorohydroquinone; alkoxy-substituted hydroquinone such as methoxy hydroquinone or ethoxy-substituted hydroquinone such as methoxy hydroquinone or ethoxy hydroquinone; aminophenol developing agents, such as 2,4-diaminophenols and methylaminophenols; ascorbic acid developing agents such as ascorbic acid, ascorbic acid ketals and ascorbic acid derivatives, such as those described in U.S. Pat. No. 3,337,342 of Green issued Aug. 22, 1967; 3-pyrazolidone developing agents such as 1-phenyl-3-pyrazolidone; 4,4-dimethyl-1-phenyl-3-pyrazolidone and 4-methyl-4-hydroxymethyl-1-phenyl-3-pyrazolidone; and acyl derivatives of para-aminophenol such as described in British Pat. No. 1,045,303 published Oct. 12, 1966 and the like. Combinations of these developing agents can be employed, if desired.

Silver halide emulsions which can be employed with this invention can be silver chloride, silver bromide, silver bromoiodide, silver chlorobromoiodide or mixtures thereof. The emulsions can be coarse or fine-grain and can be prepared by any of the well-known procedures in emulsion making such as single-jet emulsions, double-jet emulsions, such as Lippmann, ammoniacal emulsions, thiocyanate or thioether ripened emulsions, such as those described in U.S. Pat. No. 2,222,264 of Nietz et al. issued Nov. 4, 1940; U.S. Pat. No. 3,320,069 of Illingsworth issued May 15, 1967 and U.S. Pat. No. 3,271,157 of McBride issued Sept. 6, 1966. Surface image emulsions can be used or internal image emulsions such as those described in U.S. Pat. No. 2,592,250 of Davey et al. issued Apr. 8, 1952; U.S. Pat. No. 3,206,313 of Porter et al. issued Sept. 14, 1965; U.S. Pat. No. 3,367,778 of Berriman et al. issued Feb. 6, 1968; and Belgian Pat. No. 704,255. If desired, mixtures of surface and internal image emulsions can be used, as described in U.S. Pat. No. 2,996,382 of Luckey et al. issued Aug. 15, 1961. Negative type emulsions can be used or direct positive emulsions such as those described in U.S. Pat. No. 2,184,013 of Leermakers issued Dec. 19, 1939; U.S. Pat. No. 2,541,472 of Kendall et al. issued Feb. 13, 1951; U.S. Pat. No. 3,367,778 of Berriman et al. issued Feb. 6, 1968; British Pat. 723,019; French Pat. No. 1,520,821; U.S. Pat. No. 2,563,785 of Ives issued Aug. 7, 1951; U.S. Pat. No. 2,456,953 of Knott et al. issued Dec. 21, 1958 and U.S. Pat. No. 2,861,885 of Land issued Nov. 25, 1958. The emulsions can be regular grain emulsions such as those described in Klein and Moisar, *Journal of Photographic Science*, Volume 12, No. 5, September–October, 1964, pages 242–251.

The silver halide emulsions employed in the practice of the invention can be unwashed or washed to remove soluble salts. In the latter case the soluble salts can be removed by chill-setting and leaching or the emulsion can be coagulation washed.

The silver halide emulsions employed in the practice of the invention can be sensitized with chemical sensitizers, such as with reducing agents; silver, selenium, or tellurium compounds; gold, platinum or palladium compounds; or combinations of these. Suitable procedures are described, for example, in U.S. Pat. No. 1,623,499 of Shepard issued Apr. 5, 1927; U.S. Pat. No. 2,399,083 of Waller et al. issued Apr. 23, 1946; U.S. Pat. No. 3,297,447 of McVeigh issued Jan. 10, 1967 and U.S. Pat. No. 3,297,446 of Dunn issued Jan. 10, 1967.

The silver halide emulsions and/or processing compositions employed in the practice of the invention can contain speed increasing compounds such as polyalkylene glycols, cationic surfactants and thioethers or combinations of these as described, for example, in U.S. Pat. No. 2,886,437 of Piper issued May 12, 1959; U.S. Pat. No. 3,046,134 of Dann et al. issued July 24, 1962; U.S. Pat. No. 2,944,900 of Carroll et al. issued July 12, 1960 and U.S. Pat. No. 3,294,540 of Goffe issued Dec. 27, 1966.

The described silver halide emulsions employed in the practice of the invention can be protected against the production of fog and can be stabilized against loss of sensitivity during keeping. Suitable antifoggants and stabilizers each used alone or in combination include, for example, thiazolium salts; azaindenes, mercury salts as described, for example, in U.S. Pat. No. 2,728,663

of Allen et al. issued Dec. 27, 1955; urazoles; sulfocatechols; oximes described, for example, in British Pat. No. 623,448; nitron; nitroindazoles; mercaptotetrazoles; polyvalent metal salts described, for example, in U.S. Pat. No. 2,839,405 of Jones issued June 17, 1958; palladium, platinum and gold salts described, for example, in U.S. Pat. No. 2,566,263 of Trevelli et al. issued Aug. 28, 1951 and U.S. Pat. No. 2,597,915 of Yutzy et al. issued May 27, 1952.

10 The photographic and other hardenable layers of a photographic element used in the practice of the invention can be hardened by various organic or inorganic hardeners alone or in combination, such as aldehyde hardeners and blocked aldehydes, ketones, carboxylic and carbonic acid derivatives, sulfonate esters, sulfonyl halides and vinyl sulfones, active halogen compounds, epoxy compounds, aziridines, active olefins, isocyanates, carbodiimides, mixed function hardeners and polymeric hardeners such as oxidized polysaccharides such as dialdehyde starch and oxyguargum and the like.

15 A photographic element and emulsions described in the practice of the invention can contain various colloids alone or in combination as vehicles, binding agents and in various layers. Suitable hydrophilic materials include those naturally occurring substances such as proteins, for example, gelatin, gelatin derivatives, cellulose derivatives, polysaccharides such as dextran, gum arabic and the like; and synthetic polymeric substances such as water-soluble polyvinyl compounds like poly(vinylpyrrolidone), acrylamide polymers and the like.

20 The described photographic emulsion layers and other layers of the photographic element employed in the practice of the invention can also contain, alone or in combination with hydrophilic, water-permeable colloids, other synthetic polymeric compounds such as dispersed vinyl compounds, such as in latex form, and particularly those which increase the dimensional stability of the photographic materials. Suitable synthetic polymers include those described in U.S. Pat. No. 3,142,586 of Nottorf issued July 28, 1964; U.S. Pat. No. 3,193,386 of White issued July 6, 1965; U.S. Pat. No. 3,062,674 of Houck et al. issued Nov. 6, 1962; U.S. Pat. No. 3,220,844 of Houck et al. issued Nov. 30, 1965; U.S. Pat. No. 3,287,289 of Ream et al. issued Nov. 22, 1966 and U.S. Pat. No. 3,411,911 of Dykstra issued Nov. 19, 1968. Particularly effective are those water-insoluble polymers of alkyl acrylates and methacrylates, acrylic acid, sulfoalkyl acrylates or methacrylates, and those which have crosslinking sites which facilitate hardening or curing as well as those having recurring sulfobetaine units as described in Canadian Pat. No. 774,054.

25 The photographic elements employed in the practice of the invention can contain antistatic or conducting layers. Such layers can comprise soluble salts such as chloride, nitrate and the like evaporated metal layers, ionic polymers such as those described in U.S. Pat. No. 2,861,056 of Minsk issued Nov. 18, 1958 and U.S. Pat. No. 3,206,312 of Sterman et al. issued Sept. 14, 1965 or insoluble organic salts such as those described in U.S. Pat. No. 3,428,451 of Trevoy issued Feb. 18, 1969.

30 The photographic emulsions and other layers of a photographic element employed in the practice of the invention and described herein can be coated on a wide variety of supports. Typical supports include cellulose

nitrate film, cellulose ester film, poly(vinylacetal) film, polystyrene film, poly(ethylene terephthalate) film, polycarbonate film and related films or resinous materials as well as glass, paper, metal and the like. Typically a flexible support is employed, especially a paper support which can be partially acetylated or coated with baryta and/or an alpha olefin polymer, particularly a polymer of an alpha olefin containing two to 10 carbon atoms such as polyethylene, poly-propylene, ethylene-butene copolymers and the like.

The photographic elements employed in the practice of the invention can contain plasticizers and lubricants such as polyalcohols, glycerin and diols as described, for example, in U.S. Pat. No. 2,960,404 of Milton et al. issued Nov. 1, 1966; fatty acids or esters such as described in U.S. Pat. No. 2,588,765 of Robijns issued Mar. 11, 1952; and U.S. Pat. No. 3,121,160 of Duane issued Feb. 11, 1964; and silicone resins such as those described in British Pat. No. 955,061.

The photographic elements employed in the practice of the invention can contain surfactants such as saponin, anionic compounds, such as alkyl aryl sulfonates described, for example, in U.S. Pat. No. 2,600,831 of Baldsiefen issued June 17, 1962 and amphoteric compounds such as those described in U.S. Pat. No. 3,133,816 of Ben-Ezra issued May 19, 1964.

The photographic elements employed in the practice of the invention can contain matting agents such as starch, titanium dioxide, zinc oxide, silica, and polymeric beads including beads described, for example, in U.S. Pat. No. 2,992,101 of Jelley et al. issued July 11, 1961 and U.S. Pat. No. 2,701,245 of Lynn issued Feb. 1, 1955.

The described photographic elements employed in the practice of the invention can also contain brightening agents including stilbene, triazine, oxazole, and/or coumarin brightening agents. Water-soluble brighteners such as those described in German Pat. No. 972,067 and U.S. Pat. No. 2,933,390 of McFall et al. issued Apr. 19, 1960 or dispersions of brighteners can be used such as those described in German Pat. No. 1,150,274 and U.S. Pat. No. 3,406,070 of Oetiker et al. issued Oct. 15, 1968 and French Pat. No. 1,530,244.

The photographic silver halide emulsions employed in the practice of the invention can be X-ray or other nonspectrally sensitized emulsions or they can contain spectral sensitizing dyes. The photographic silver halide emulsions can conveniently be ortho-sensitized or pan-sensitized with spectral sensitizing dyes. For instance, these emulsions can be spectrally sensitized by treating with a solution of a sensitizing dye in an organic solvent or the dye can be added in the form of a dispersion such as described in French Pat. No. 1,482,774. Spectral sensitizing dyes useful in sensitizing such emulsions are described, for example, in U.S. Pat. No. 2,526,632 of Brooker et al. issued Oct. 24, 1950; U.S. Pat. No. 2,503,776 of Sprague issued Apr. 11, 1950; U.S. Pat. No. 2,493,748 of Brooker et al. issued Jan. 10, 1950; and U.S. Pat. No. 3,384,486 of Taber et al. issued May 21, 1968. Spectral sensitizers which can be used include the cyanines, merocyanines, complex (trinuclear or tetrานuclear) cyanines, complex (trinuclear or tetrานuclear) merocyanines, holopolar cyanines, styryls, hemicyanines, such as enamine hemicyanines, oxonols and hemioxonols. Dyes of the cyanine classes can contain such basic groups as the thiazolines, oxazolines, pyrrolines, pyridines, oxa-

zoles, thiazoles, selenazoles and imidazoles. Such groups can contain alkyl, alkylene, hydroxyalkyl, sulfoalkyl, carboxyalkyl, aminoalkyl and enamine substituents and can be fused to carbocyclic or heterocyclic ring systems either unsubstituted or substituted with halogen, phenyl, alkyl, haloalkyl, cyano or alkoxy groups. The dyes can be symmetrical or unsymmetrical and can contain alkyl, phenyl, enamine or heterocyclic substituents on the methine or polymethine chain. The

merocyanine dyes can contain the basic groups described as well as acid groups such as thiohydantoins, rhodanines, oxazolidenediones, thiazolidenediones, barbituric acids, thiazolineones and malononitrile. These acid groups can be substituted with alkyl, alkylene, phenyl, carboxyalkyl, sulfoalkyl, hydroxyalkyl, alkoxyalkyl, alkylamino groups or heterocyclic groups. Combinations of these dyes can be used if desired. In addition, supersensitizing addenda which do not absorb visible light can be included, such as ascorbic acid derivatives, azaindenes, cadmium salts and organic sulfonic acids as described in U.S. Pat. No. 2,933,390 of McFall et al. issued Apr. 19, 1960 and U.S. Pat. No. 2,937,089 of Jones et al. issued May 17, 1960.

The various layers including the photographic emulsion layer of the photographic element employed in the practice of the invention can contain light absorbing materials and filter dyes such as those described in U.S. Pat. No. 3,253,921 of Sawdey issued May 31, 1966; U.S. Pat. No. 2,274,782 of Gaspar issued Mar. 3, 1942; U.S. Pat. No. 2,527,583 of Silberstein et al. issued Oct. 31, 1950 and U.S. Pat. No. 2,956,879 of VanCampen issued Oct. 18, 1960. If desired, the dyes can be mordanted, for example, as described in U.S. Pat. No. 3,282,699 of Jones et al. issued Nov. 1, 1966.

The sensitizing dyes and other addenda used in the practice of the invention can be added from water solutions or suitable organic solvent solutions can be used. The compounds can be added using various procedures including those described in U.S. Pat. No. 2,912,343 of Collins et al. issued Nov. 10, 1959; U.S. Pat. No. 3,342,605 of McCrossen et al. issued Sept. 19, 1967; U.S. Pat. No. 2,996,287 of Audran issued Apr. 15, 1961 and U.S. Pat. No. 3,425,835 of Johnson et al. issued Feb. 4, 1969.

The following examples are included for a further understanding of the invention.

#### EXAMPLE 1

This example illustrates use of the combination of the described disulfones with a hydroxylamine silver halide developing agent and producing a positive image in a photographic chemical transfer system.

A processing composition is prepared by mixing the following components.

|                                                                                                          |         |
|----------------------------------------------------------------------------------------------------------|---------|
| Stock solution A (850 ml water, 213.2 g.<br>potassium hydroxide with 0.16 g.<br>4-thiazolidine-2-thione) | 45.0 ml |
| Bis(methylsulfonyl)methane                                                                               | 1.65 g  |
| N-N-Diethylhydroxylamine                                                                                 | 2.5 ml  |
| 60 Hydroxyethylcellulose (Natrasol 250H<br>sold by Hercules Powder Co., U.S.A.)                          | 1.35 g  |

A layer of this processing composition about 0.001-inch in thickness is spread between a sensitometrically exposed photographic element containing a fine-grain, negative-type, developing out, gelatino silver bromoiodide emulsion layer on a film support and a receiving sheet containing palladium development nuclei. The

processing composition is spread between the photographic element and the image receiver so as to have the image and receiver contact the processing composition simultaneously. After 30 seconds contact time at 22°C the photographic element with the processing layer is stripped away from the image receiver. A positive image of good discrimination is observed on the image receiver. The minimum reflection density of the image on the image receiver is 0.08 and the maximum reflection density of this image is 1.69.

#### EXAMPLE 2

This is a comparative example.

The procedure set out in Example 1 is repeated with the exception that 1.08 grams of uracil is employed in place of bis(methylsulfonyl)methane. A transfer image is produced having a minimum reflection density of 0.10 and a maximum reflection density of 0.79.

#### EXAMPLE 3

This is a comparative example.

The procedure set out in Example 1 is repeated with the exception that 2.38 grams of sodium thiosulfate pentahydrate is employed in place of bis(methylsulfonyl)methane. A transfer image is produced on the image receiver having a minimum reflection density of 0.30 and a maximum reflection density of 0.57.

#### EXAMPLE 4

This is a comparative example.

The procedure set out in Example 1 is repeated with the exception that 0.93 grams of potassium thiocyanate is employed in place of the bis(methylsulfonyl)methane. A transfer image is produced on the image receiver having a minimum reflection density of 0.10 and a maximum reflection density of 0.16.

#### EXAMPLE 5

This is a comparative example.

The procedure set out in Example 1 is repeated with the exception that 1.10 ml of an 80 percent by weight aqueous mercaptoacetic acid solution is employed in place of the bis(methylsulfonyl)methane. A transfer image is produced on the image receiver having a minimum reflection density of 0.10 and a maximum reflection density of 0.10. This indicates no satisfactory image transfer.

#### EXAMPLE 6

This is a comparative example.

The procedure set out in Example 1 is repeated with the exception that 1.69 grams of cysteine hydrochloride monohydrate is employed in place of the bis(methylsulfonyl)-methane. No satisfactory image transfer is observed.

#### EXAMPLE 7

This is a comparative example.

The procedure set out in Example 1 is repeated with the exception that 3.10 grams of hydroquinone is employed in place of the N,N-diethylhydroxylamine. An image transfer is observed on the image receiver having a minimum reflection density of 0.20 and a maximum reflection density of 1.10.

#### EXAMPLE 8

This is a comparative example.

The procedure set out in Example 1 is repeated with the exception that 4.98 grams of D-(-)-arabooascorbic acid is employed in place of the N,N-diethylhydroxylamine. A transfer image is produced on the image receiver having a minimum reflection density of 0.16 and a maximum reflection density of 0.86.

#### EXAMPLE 9

This examples illustrates image stability of the image produced according to Example 1.

A print as produced according to Example 1 is subjected to the following conditions:

|    | Identification  | Treatment Condition                                                            |
|----|-----------------|--------------------------------------------------------------------------------|
| 15 | Fresh           | 22°C., about 50% relative humidity, no light                                   |
|    | Light Incubated | 38°C., about 90% relative humidity, 1800 foot-candles fluorescent illumination |

20 After 48 hours at the described conditions, sensitometric curves are plotted for the fresh and light incubated samples. The following Table I indicates the stability of prints produced according to Example 1 as measured by the gain in speed at a density of 0.20.

TABLE I

#### Relative Speed at 0.2 Density (Log E)

| Fresh Speed | Light Incubated |      |
|-------------|-----------------|------|
|             | Speed           | Gain |
| 1.00        | 1.04            | 0.04 |

30 This data indicates that very little loss of image is produced upon incubation.

#### EXAMPLE 10

35 This example illustrates that various processing layer thicknesses can be employed without adversely affecting the developed image according to the invention.

The procedure set out in Example 1 is repeated but with varying processing layer thickness. Processing layer thicknesses of 0.0007-inch, 0.0010-inch and 0.0013-inch are employed. The photographic speed, i.e., Log E, and contrast, i.e., bar gamma are observed employing the different processing layer thicknesses. The following is observed.

TABLE II

| Developer Layer Thickness | Relative Speed Log E (at 0.2 Density) | Contrast Bar Gamma |
|---------------------------|---------------------------------------|--------------------|
| 0.0007 inch               | 1.00                                  | 1.67               |
| 0.0010 inch               | 1.00                                  | 1.68               |
| 0.0013 inch               | 0.97                                  | 1.58               |

50 This illustrates that the photographic speed and contrast change very little with processing layer thickness employing a combination according to the invention.

55 Results similar to those of Example 1 are obtained in each of the following Examples 11—25 using the noted hydroxylamine silver halide developing agents in place of N,N-diethylhydroxylamine.

#### EXAMPLE 11

##### Hydroxylamine

#### EXAMPLE 12

##### N-methylhydroxylamine

#### EXAMPLE 13

##### N-ethylhydroxylamine

## EXAMPLE 14

N-propylhydroxylamine

## EXAMPLE 15

N-isopropylhydroxylamine

## EXAMPLE 16

N,N-dimethylhydroxylamine

## EXAMPLE 17

N-methyl-N-propylhydroxylamine

## EXAMPLE 18

N-ethyl-N-propylhydroxylamine

## EXAMPLE 19

N,N-diisopropylhydroxylamine

## EXAMPLE 20

N,N-dimethylhydroxylamine

## EXAMPLE 21

N-ethyl-N-hydroxyethylhydroxylamine

## EXAMPLE 22

N-hydroxyethyl-N-carboxyethylhydroxylamine

## EXAMPLE 23

N,N-di-(methoxyethyl) hydroxylamine

## EXAMPLE 24

N,N-di-(2-ethoxyethyl) hydroxylamine

## EXAMPLE 25

N,N-di-(2-methoxyethoxyethyl) hydroxylamine

Results similar to those of Example 1 are obtained in each of the following Examples using the noted 1,1-bis(sulfonyl)alkane silver halide solubilizing agent in place of bis(methylsulfonyl) methane.

## EXAMPLE 26

1,1-Bis-(methylsulfonyl)ethane

## EXAMPLE 27

1,1-Bis-(ethylsulfonyl)ethane

## EXAMPLE 28

1,1-Bis-(methylsulfonyl)propane

## EXAMPLE 29

1-ethylsulfonyl-1-methylsulfonylmethane

## EXAMPLE 30

1-ethylsulfonyl-1-methylsulfonylthane

## EXAMPLE 31

1,1-Bis-(beta-hydroxyethylsulfonyl)methane

## EXAMPLE 32

1,1-Bis-(carboxymethylsulfonyl)methane

## EXAMPLE 33

1,1-Bis-(beta-carboxyethylsulfonyl)methane

## EXAMPLE 34

The procedure set out in Example 1 is repeated with

the exception that the processing composition described in Example 1 is replaced with the following processing composition:

|    |                                                                           |          |
|----|---------------------------------------------------------------------------|----------|
| 5. | Water                                                                     | 850.0 ml |
|    | Potassium hydroxide                                                       | 80.0 g   |
|    | Bis(methylsulfonyl)methane                                                | 33.0 g   |
|    | p-Methylaminophenol sulfate                                               | 10.0 g   |
|    | N,N-diethyl hydroxylamine                                                 | 17.0 ml  |
|    | 4-Thiazolidine-b 2-thione                                                 | 0.2 g    |
| 10 | Hydroxyethylcellulose (Natrasol 250H sold by Hercules Powder Co., U.S.A.) | 27.0 g   |

A positive image is produced having a neutral black tone. The positive image has a minimum reflection density of 0.07 and a maximum reflection density of 1.7.

15 This example illustrates the use of an auxiliary silver halide developing agent. The processing composition of this example is also less alkaline than the processing composition of Example 1.

The invention has been described in detail with particular reference to preferred embodiments thereof, 20 but it will be understood that variations and modifications can be effected within the spirit and scope of the invention.

What is claimed is:

25 1. A photographic element comprising a support, photographic silver halide, a 1,1-bis-sulfonyl alkane silver halide solubilizing agent with a hydroxylamine silver halide developing agent.

30 2. A photographic element as in claim 1 comprising a support, photographic silver halide, bis(methylsulfonyl)-methane and N,N-diethylhydroxylamine.

35 3. In a photographic diffusion transfer product comprising in combination (a) a photographic element comprising photographic silver halide, (b) a processing composition comprising a silver halide solubilizing agent and (c) an image-receiving layer, said product containing a silver halide developing agent, the improvement comprising a 1,1-bis-sulfonyl alkane as said silver halide solubilizing agent and a hydroxyl-amine silver halide developing agent as said developing agent.

40 4. The photographic diffusion transfer product of claim 3 wherein said 1,1-bis-sulfonyl alkane is a compound of the formula:



45 wherein  $R_1$  and  $R_2$  each represent an alkyl group containing one to four carbon atoms and  $R_3$  represents hydrogen or an alkyl group containing one to four carbon atoms, and said hydroxylamine silver halide developing agent is a compound of the formula:



55 wherein  $R_4$  and  $R_5$  are each hydrogen, alkyl containing one to four carbon atoms, alkoxyalkyl containing three to six carbon atoms, or alkoxyalkoxyalkyl containing five to 10 carbon atoms.

60 5. The photographic diffusion transfer product of claim 3 wherein said 1,1-bis-sulfonyl alkane is bis-(methylsulfonyl)methane and said hydroxylamine silver halide developing agent is N,N-diethylhydroxylamine.

65 6. The photographic diffusion transfer product of claim 3 wherein said 1,1-bis-sulfonyl alkane and said hydroxylamine are present in said processing composition.

7. The photographic diffusion transfer product of claim 3 wherein said diffusion transfer product also comprises an auxiliary silver halide developing agent.

8. The photographic diffusion transfer product of claim 3 wherein said diffusion transfer product also comprises an auxiliary silver halide developing agent which comprises an aminophenol silver halide developing agent.

9. In a photographic diffusion transfer process comprising developing a latent image in a photographic diffusion transfer product comprising (a) a photographic element comprising photographic silver halide, (b) a processing composition comprising a silver halide solubilizing agent and (c) an image receiving layer, said product also comprising a silver halide developing agent, and forming an imagewise distribution of a silver complex in said element by contacting undeveloped silver halide in said element with said silver halide solubilizing agent and transferring at least part of the silver complex to said image receiver layer, the improvement comprising employing a 1,1-bis-sulfonyl alkane as said silver halide solubilizing agent and hydroxylamine as said silver halide developing agent.

10. The photographic diffusion transfer process of claim 9 wherein said 1,1-bis-sulfonyl alkane is a compound of the formula:



10

5

wherein R<sub>1</sub> and R<sub>2</sub> each represent an alkyl group containing one to four carbon atoms and R<sub>3</sub> represents hydrogen or an alkyl group containing one to four carbon atoms, and said hydroxylamine silver halide developing agent is a compound of the formula:

wherein R<sub>4</sub> and R<sub>5</sub> are each hydrogen, alkyl containing one to four carbon atoms, alkoxyalkyl containing three to six carbon atoms, or alkoxyalkoxyalkyl containing five to 10 carbon atoms.

11. The photographic diffusion transfer process of claim 9 wherein said 1,1-bis-sulfonyl alkane is bis(methyl-sulfonyl)methane and said hydroxylamine silver halide developing agent is N,N-diethylhydroxylamine.

12. The photographic diffusion transfer process of claim 9 wherein said processing composition also comprises an auxiliary silver halide developing agent.

13. The photographic diffusion transfer process of claim 9 wherein said processing composition also comprises an auxiliary silver halide developing agent which comprises an aminophenol silver halide developing agent.

\* \* \* \* \*

30

35

40

45

50

55

60

65

UNITED STATES PATENT OFFICE  
CERTIFICATE OF CORRECTIONPatent No. 3,770,432Dated November 6, 1973Inventor(s) Donald G. Yungkurth and Gary J. McSweeney

It is certified that error appears in the above-identified patent  
and that said Letters Patent are hereby corrected as shown below:

The title "A Photographic Composition of 1,1-Bis-Sulfonyl Alkane and Hydroxylamine" should read  
---Photographic Composition of 1,1-Bis-Sulfonyl Alkane  
and Hydroxylamine---.

Column 1, line 55, "agent" should read ---agents---.

Column 5, line 17, "lay" should read ---layer---.

Line 45, "photographic" should read ---photographic---.

Column 6, line 35, "a" should be inserted  
after "of". Line 65, "1,1-bis-sulfony" should read  
---1,1-bis-sulfonyl---.

Column 8, line 53, after "ethoxy" delete  
"substituted". Lines 54-55, after "hydroquinone" delete  
"such as methoxy hydroquinone or ethoxy hydroquinone".

Column 13, line 39, "comparative" should read  
---comparative---. Line 62, "obsreve" should read  
---observed---.

Column 16, line 8, "4-Thiazolidine- $\beta$ 2-thione"  
should read ---4-Thiazolidine-2-thione---.

In the Claims:

Column 17, line 22, after "and" insert "a".

Signed and sealed this 1st day of October 1974.

(SEAL)

Attest:

By M. GIBSON JR.  
Acting OfficerC. MARSHALL DANN  
Commissioner of Patents